# EUROPEAN PATENT SPECIFICATION

(11) **EP 1 621 604 B1**
(45) Date of publication and mention of the grant of the patent: **01.10.2008**
(21) Application number: 05425530.2
(22) Date of filing: 22.07.2005
(51) Int. Cl.: C11D 3/00, C11D 17/04, C11D 3/37, C11D 3/22

(54) **Colour scavenger material**
Material zum Auffangen von Farbstoffen
Matériau de capture de couleurs

(30) Priority: 29.07.2004 WO PCT/IT2004/000419
(43) Date of publication of application: 01.02.2006
(73) Proprietor: Orlandi S.p.A., 20122 Milano (IT)
(72) Inventor: Orlandi, Vittorio, 20122 Milano (IT)
(74) Representative: Long, Giorgio

(56) References cited:
- EP-A- 1 083 218
- WO-A-99/15614
- WO-A-20/04067691
- US-A1- 2002 119 721
- US-A1- 2003 118 730

## Description

This invention relates to a material for removing excess colour in washing water and a method for its production.

It is known that the majority of "coloured" garments loose a certain amount of colour in washing water, and must therefore be washed separately from "white" garments, to prevent them from becoming partially or totally coloured.

This has created a problem for housewives all over the world, and has always been resolved by carefully separating "whites" from "coloureds", using low temperature washing machine programmes, or by trying to make pigments more suitable for the fabrics.

In all these cases, the desired results are not always obtained, and very often after a machine wash, some of the "whites" are partially or totally coloured.

This invention faces the problem from another viewpoint, in other words, it provides a material that is able to totally eliminate any colour present in washing water, thus preventing the dying of the "white" garments. Consequently, the "coloureds" and "whites" can be washed in the machine at the same time in the presence of the material of the present invention which acts as a "dye scavenger".

The present invention relates to a material comprising a non-woven substrate and a suitable additive that removes the colour.

The substrate can have any form and size, such as, for example a handkerchief or a piece of cloth. Preferably, the substrate has the form of a handkerchief. The substrate is 100% regenerated cellulose, for example: lyocell^{®} (that is regenerated cellulose fibre, obtained using a process of dissolving and spinning in organic solvent) or tencell^{®}. The substrate is 100% regenerated cellulose obtained using the spunlaced technique.

The substrate performs the function of "carrier" of the additive, which removes the colour.

The additive is a substance that has a very high affinity for colourants. In fact the principle at the base of this invention is the fact that the colourant released in the washing water by the coloured garments has a greater affinity for the material of the present invention than for the fabric of the "whites". The additive is a cationic heterocyclic polymer, the COBRAL MM marketed by the company, Lamberti S.p.A..

The material object of the present invention can be obtained by combining in any manner, the substrate with the additive.

The substrate preferably has a weight that ranges between 150 grams/m² and 50 grams/m², more preferably between 100 grams/m² and 60 grams/m². The fibres of the substrate preferably have a size that ranges between 0,5 dtex and 5 dtex, preferably between 1 dtex and 2 dtex.

The additive is fixed on and/or incorporated into the substrate by means of: impregnation, spraying, printing and/or plating and the relation existing between the additive and the substrate can be: absorption, adsorption, hydrogen bonding, electrostatic force for example ion/ion interaction or ion/dipole interaction, incorporation, chemical or physical bonds, etc.

Under another aspect, the present invention relates to a process for the production of the dye scavenger.

Said process comprises the following steps:
a) Provide the substrate described above;
b) Process the substrate with the additive described above;
c) Pass the processed substrate through two or more rollers in order to remove any excess additive;
d) Dry the substrate.

In step b) the substrate is preferably processed by means of impregnation, spraying, printing and/or plating, all of which are techniques known to the art. Preferably, the additive is applied by spraying and/or impregnation, and more preferably by impregnation.

In the case where impregnation techniques are used, the substrate is passed through a solution of the additive having a suitable concentration in order to leave on the finished material an amount of additive ranging between 0,5% and 50% in weight on the finished material, preferably between 5% and 25%, more preferably between 10% and 22%.

The additive solution is preferably an aqueous solution made alkaline by the addition of a base, preferably NaOH. The concentration of the base ranges between 5 and 100 grams/litre, preferably between 8 and 50 grams/litre, more preferably between 10 and 30 grams/litre. The additive concentration generally ranges between 5 grams/litre and 300 grams/litre, preferably between 25 grams/litre and 200 grams/litre, more preferably between 100 grams/litre and 180 grams/litre.

In step c), the substrate is passed through two or more rollers and pressed in order to eliminate any excess additive and to leave on the substrate the required amount (foulard technique). The pressing pressure will depend on the amount of additive to be left in the finished material and on the concentration of the solution or the additive as applied during stage a).

The steps a) and b) and c) can be performed at any suitable temperature that does not alter the properties of the substrate and the additive, preferably at room temperature.

During stage d), the substrate is dried, preferably in an oven, at a temperature ranging between 100°C and 220°C, preferably between 130°C and 180°C, for a period of time that depends on the amount of additive and solvent present, on the temperature and the efficiency of the drying system.

For example, in order to obtain a material that contains an amount of additive ranging between 5% and 25%, using additive solutions with a concentration between 100 grams/litre and 180 grams/litre, pressing can be applied at a pressure ranging between 0,5 and 5 bar, preferably approximately 2 bar and drying can be performed at a temperature ranging between 130°C and 180°C, for a period of time between 1 and 5 minutes, preferably approximately 3 minutes.

The aforesaid parameters can be easily modified by those skilled in the art according to the final material that is required (that is with a greater or lesser amount of impregnated additive) and the machines that are available. For example, if a very efficient oven is available, the drying time can be reduced considerably, thus speeding up the whole process; if the foulard technique is used wherein pressing is performed using three cylinders, the applied pressure could be less than that used when pressing with two cylinders, etc.

The process should be preferably performed continuously, that is, the substrate is subjected to impregnation, pressing and drying without any intermediate stages or pauses (possibly to permit the additive to bond better with the substrate) between one process and another. All this is possible because the additive possesses a very high affinity for the substrate and, therefore the required amount of additive bonds with the substrate almost instantly and it is not necessary that the substrate be left to impregnate for a long period of time.

The dye scavenger material of the present invention is normally introduced into conventional domestic or professional washing machines before the beginning of the washing cycle together with the "white" and "coloured" laundry.

The term, "whites" refers to a laundry wash comprising white and light coloured fabrics (for example: beige, pale pink, pale blue, grey etc.); preferably light coloured fabrics.

The term "coloureds" refers to a laundry wash comprising strongly coloured fabrics (for example: red, bordeaux, yellow etc.) or very dark colours (for example: navy blue, black, dark green, denim etc.). These fabrics can be new or can have already been subjected to washing in a washing machine. Preferably, by "coloureds" the term refers to a laundry wash comprising strongly coloured fabrics (for example: red, bordeaux, yellow, orange, etc.); and more preferably this refers to strongly coloured fabrics that have been previously washed 5 or 6 times.

Ideally, the material of the invention is introduced into the washing machine together with light coloured and strongly coloured fabrics coloured fabrics that have already been previously washed 5 or 6 times. The number of material sheets of the invention that are used for each wash will depend on the weight of laundry and the colours present. Preferably, 2 or more sheets of the material of the invention are introduced into the washing machine in the case of fabrics that loose a large amount of colour, for example cotton fabrics with strong intense colours.

The material of the invention is resistant to normal washing temperatures and common detergents and additives, including bleach, and can be used repeatedly several times before loosing its efficacy.

### EXAMPLE I

A solution is prepared mixing 1 litre of water with 150 grams of COBRALL MM and 20 grams of NaOH 36°be. A piece of 100% lyocell^{®} non-woven fabric with a weight of 70 grams/m² is passed in a continuous manner, through a bath containing the aforesaid solution so that it is well impregnated, then passed through two rollers that press the material at a pressure of 2 bar, and finally through a cylinder oven, where it is dried at 150°C for 3 minutes. The amount of additive present on the substrate is 30% in weight based on the weight of the finished material, if the pk del foulard (that is the % of the liquid that remains in the non-woven fabric after pressing) is equal to 200%.

### EXAMPLE II

The material obtained in example I is placed in a domestic washing machine together with light coloured garments: beige and pink, and strongly coloured garments already washed 6 times: red and yellow. The garments are washed at 60°C for approximately 2 hours. During the washing cycle the water remains clear all the time, and on completion, it can be seen that there is no partial or total colouring of the light coloured garments; the colour lost by the strongly coloured garments has been retained by the dye scavenger and the material has been subjected to no alteration.

### ADVANTAGES

The material of the invention is far more resistant, especially when it is wet, than the cotton that is normally used as a substrate for this type of product. The combined action of the substrate and the additive which both possess a high affinity for the pigments, provide a very efficient capacity for retaining the colour present in the washing water, for higher than other products known in the art.

The process of the invention is very rapid in that it can be performed in a continuous manner and has a limited number of stages. This provides a considerable saving in time and energy. In fact, the final material is obtained within a few minutes since the additive is bonded with the substrate almost immediately, and it does not need to be left to rest for hours (to ensure that the additive is absorbed in the substrate) as occurs with the processes known in the art. All this is possible thanks to the use of the additives of the present invention that possess a very high affinity for the substrate and are absorbed in efficacious amounts almost immediately.

The particular preferred combination between a substrate in 100% regenerated cellulose, for example lyocell^{®}, and a cationic heterocyclic polymer, for example COBRAL MM, is the one that has allowed the best possible results in terms of resistance to conditions of use (and therefore provides the possibility of repeated use) and in terms of efficiency as a scavenger.

Therefore, the present invention provides a material and a production process higher in quality and efficiency than those described in known state of the art.

## Claims

1. Material to remove the colour released by laundry in washing water comprising a substrate and an additive **characterised in that** said substrate is a non-woven, 100% regenerated cellulose spunlaced fabric and that said additive is COBRAL MM.

2. Material according to claim 1
wherein said substrate is spunlaced lyocell.

3. Material according to 1 or 2 wherein said substrate has a weight that ranges between 150 grams/m², and 50 grams/m², preferably between 100 grams/m² and 60 grams/ m².

4. Production process for dye scavenger material according to claim 1 comprising the following stages:
a) Provide a non-woven, 100% regenerated cellulose spunlaced fabric substrate;
b) Process the substrate with COBRAL MM;
c) Eliminate any excess additive;
d) Dry the substrate.

5. Process according to claim 4 wherein, during stage b), the substrate is processed by means of impregnation, spraying, printing and/or plating.

6. Process according to claim 4 or 5 wherein, during stage b), the substrate is processed by impregnation.

7. Process according to claim 6 wherein, during stage b) in the case where the impregnation technique is used, the substrate is passed through a solution of the additive.

8. Process according to claim 7 wherein said solution of the additive is an aqueous solution made alkaline through the addition of a base, preferably NaOH.

9. Process according to claim 7 or 8 wherein the amount of the base used ranges between 5 and 100 grams/litre.

10. Process according to any one of the claims from 8 to 9
wherein the amount of base used ranges between 8 and 50 grams/litre, preferably between 10 and 30 grams/litre.

11. Process according to any one of the claims from 7 to 10
wherein the concentration of the additive ranges between 5 and 300 grams/litre.

12. Process according to any one of the claims from 7 to 11
wherein the concentration of the additive ranges between 25 and 200 grams/litre, preferably between 100 and 180 grams/litre.

13. Process according to any one of the claims from 4 to 12
wherein, during the stage c), any excess additive is removed by passing the substrate through two or more rollers.

14. Process according to any one of the claims from 4 to 13
wherein, during stage d), the substrate is dried in an oven at a temperature ranging between 100 and 220°C preferably between 130 and 180°C.

15. Process according to any one of the claims from 4 to 14
wherein, during stage d), the substrate is dried for a period of the time ranging between 1 and 5 minutes, preferably approximately 3 minutes.

16. Process according to any one of the claims from 4 to 15 that is performed in a continuous manner.

17. Material which can be obtained by means of the process according to any one of the claims from 4 to 16.

18. Use of the material according to any one of the claims from 1 to 3 to remove the colour present in the washing water of a laundry wash.

19. Method for removing colour from washing water of a laundry wash using the material according to any one of the claims from 1 to 3 comprising the following stages:
- Provide an aqueous bath containing laundry of various colours;
- Include in said bath the material according to any one of the claims from 1 to 3;
- Leave said material in said bath for a total wash cycle in a washing machine after which said material and said laundry are separated, with the result that said material has captured all the colour present in the washing water.

20. Method according to claim 19 wherein the stages are repeated many times in presence of the same material.

## Patentansprüche

1. Material, mit dem vom Waschgut in die Waschlauge freigesetzte Farbsubstanzen entfernbar sind und das ein Substrat und ein Additiv aufweist, **dadurch gekennzeichnet, dass** es sich beim Substrat um ein wasserstrahlgena-, deltes Vlies aus 100 % regenerierter Cellulose und beim Additiv um COBRAL MM handel

2. Material nach Anspruch 1. bei dem das Substrat wassersstrahlgenadeltes Lyocell ist.

3. Material nach Anspruch 1 oder 2, bei dem das Substrat ein Gewicht im Bereich von 150 g/m² und 50 g/m², vorzugsweise zwischen 100 g/m² und 60 g/m² aufweist.

4. Verfahren zur Herstellung eines Farbstoff-Absorbermaterials nach Anspruch 1 mit folgenden Stufen:
(a) Bereitstellen eines wasserstrahlgenadelten Vliessubstrats aus 100 % regenerierter Cellulose;
(b) Bearbeiten des Substrats mit COBRAL MM;
(c) Beseitigen eines Additiv-Überschusses;
(d) Trocknen des Substrats.

5. Verfahren nach Anspruch 4, in dessen Stufe (b) das Substrat durch Imprägnieren, Besprühen, Bedrucken und/oder Plattieren behandelt wird.

6. Verfahren nach Anspruch 4 oder 5, in dessen Stufe (b) das Substrat durch Imprägnieren behandelt wird.

7. Verfahren nach Anspruch 6, in dessen Stufe (b) für den Fall der Anwendung des Imprägnierens das Substrat durch eine Lösung des Additivs geführt wird.

8. Verfahren nach Anspruch 7, bei dem die Additivlösung eine wässrige, durch Zugabe einer Base - vorzugsweise NaOH - alkalisch gemachte Lösung ist.

9. Verfahren nach Anspruch 7 oder 8, bei dem die eingesetzte Menge der Base im Bereich zwischen 5 g/Liter und 100 g/Liter liegt,

10. Verfahren nach einem der Ansprüche 8 bis 9, bei dem die eingesetzte Menge der Base im Bereich zwischen 8 g / Liter und 50 g / Liter, vorzugsweise zwischen 10 g/Liter und 30 g/Liter liegt.

11. Verfahren nach einem der Ansprüche 7 bis 10, bei dem die Konzentration des Additivs im Bereich zwischen 5 g/Liter und 300 g/Liter liegt.

12. Verfahren nach einem der Ansprüche 7 bis 11, bei dem die Konzentration des Additivs im Bereich zwischen 25 g/Liter und 200 g/Liter, vorzugsweise zwischen 100 g/Liter und 180 g/Liter liegt.

13. Verfahren nach einem der Ansprüche 4 bis 12, in dessen Stufe (c) man den Additivüberschuss entfernt, indem man das Substrat zwischen zwei oder mehr Walzen hindurch schickt.

14. Verfahren nach einem der Ansprüche 4 bis 13, in dessen Stufe (d) man das Substrat in einem Ofen bei einer Temperatur im Bereich von 100 °C bis 220 °C, vorzugsweise 130 °C bis 180 °C trocknet.

15. Verfahren nach einem der Ansprüche 4 bis 14, in dessen Stufe (d) man das Substrat für die Dauer von 1 min bis 5 min, vorzugsweise etwa 3 min trocknet.

16. Verfahren nach einem der Ansprüche 4 bis 15, das man kontinuierlich durchführt.

17. Material, dass sich mittels des Verfahrens nach einem der Ansprüche 4 bis 16 erhalten lässt.

18. Anwendung des Materials nach einem der Ansprüche 1 bis 3 zum Entfernen der in der Waschlauge des Waschguts vorliegenden Farbsubstanz.

19. Verfahren zum Entfernen der in der Waschlauge von Waschgut vorliegenden Farbsubstanz unter Verwendung des Materials nach einem der Ansprüche 1 bis 3 mit folgenden Stufen:
- Bereitstellen eines wässrigen Bades mit verschiedenfarbigem Waschgut; -
Einbringen des Materials nach einem der Ansprüche 1 bis 3 in das Bad; und
- Belassen des Materials im Bad für die Dauer eines vollständigen Waschzyklus in einer Waschmaschine, wonach man das Material und das Waschgut trennt mit dem Ergebnis, dass das Material die gesamte Farbsubstanz in der Waschlauge aufgenommen hat.

20. Verfahren nach Anspruch 19, dessen Stufen man in Gegenwart des gleichen Materials mehrfach wiederholt.

## Revendications

1. Matière pour éliminer la couleur libérée par le linge dans l'eau de lavage, comprenant un substrat et un additif, **caractérisée en ce que** ledit substrat est une étoffe entrelacée par filage non tissée, à 100 % de cellulose régénérée, et **en ce que** ledit additif est le COBRAL MM.

2. Matière suivant la revendication 1, dans laquelle ledit substrat consiste en Lyocell entrelacé par filage.

3. Matière suivant la revendication 1 ou 2, dans laquelle ledit substrat a un poids qui est compris entre 150 g/m² à 50 g/m², de préférence entre 100 g/m² et 60 g/m².

4. Procédé pour la production d'une matière fixant les colorants suivant la revendication 1, comprenant les étapes suivantes :
a) fourniture d'un substrat consistant en une étoffe entrelacée par filage non tissée, à 100 % de cellulose régénérée ;
b) traitement du substrat avec du COBRAL MM ;
c) élimination de tout excès d'additif ;
d) séchage du substrat.

5. Procédé suivant la revendication 4, dans lequel, au cours de l'étape b), le substrat est traité par imprégnation, pulvérisation, impression et/ou placage.

6. Procédé suivant la revendication 4 ou 5, dans lequel, au cours de l'étape b), le substrat est traité par imprégnation.

7. Procédé suivant la revendication 6, dans lequel, au cours de l'étape b), dans le cas où la technique d'imprégnation est utilisée, le substrat est passé à travers une solution de l'additif.

8. Procédé suivant la revendication 7, dans lequel ladite solution de l'additif est une solution aqueuse rendue alcaline par addition d'une base, de préférence de NaOH.

9. Procédé suivant la revendication 7 ou 8, dans lequel la quantité de base utilisée est comprise entre 5 et 100 g/l.

10. Procédé suivant l'une quelconque des revendications 8 à 9, dans lequel la quantité de base utilisée est comprise entre 8 et 50 g/l, de préférence entre 10 et 30 g/l.

11. Procédé suivant l'une quelconque des revendications 7 à 10, dans lequel la concentration de l'additif est comprise entre 5 et 300 g/l.

12. Procédé suivant l'une quelconque des revendications 7 à 11, dans lequel la concentration de l'additif est comprise entre 25 et 200 g/l, de préférence entre 100 et 180 g/l.

13. Procédé suivant l'une quelconque des revendications 4 à 12, dans lequel, au cours de l'étape c), tout excès d'additif est éliminé en faisant passer le substrat entre deux ou plus de deux rouleaux.

14. Procédé suivant l'une quelconque des revendications 4 à 13, dans lequel, au cours de l'étape d), le substrat est séché dans un four à une température comprise entre 100 et 220°C, de préférence entre 130 et 180°C.

15. Procédé suivant l'une quelconque des revendications 4 à 14, dans lequel, au cours de l'étape d), le substrat est séché pendant une période de temps allant de 1 à 5 minutes, de préférence d'approximativement 3 minutes.

16. Procédé suivant l'une quelconque des revendications 4 à 15, qui est mis en oeuvre de manière continue.

17. Matière qui peut être obtenue au moyen du procédé suivant l'une quelconque des revendications 4 à 16.

18. Utilisation de la matière suivant l'une quelconque des revendications 1 à 3 pour éliminer la couleur présente dans l'eau de lavage d'un lavage du linge.

19. Procédé pour éliminer la couleur de l'eau de lavage d'un lavage du linge en utilisant la matière suivant l'une quelconque des revendications 1 à 3, comprenant les étapes suivantes :
- fournir un bain aqueux contenant du linge de diverses couleurs ;
- incorporer audit bain la matière suivant l'une quelconque des revendications 1 à 3 ;
- laisser ladite matière dans ledit bain pendant un cycle total de lavage dans une machine à laver, puis ladite matière et ledit linge sont séparés, avec pour résultat la capture par ladite matière de la totalité de la couleur présente dans l'eau de lavage.

20. Procédé suivant la revendication 19, dans lequel les étapes sont répétées de nombreuses fois en présence de la même matière.
